

May 31, 1932.

J. E. LITTLE ET AL

1,860,811

TREATMENT OF ORES

Filed May 26, 1926

2 Sheets-Sheet 1

*Fig. 1.*



*Fig. 2.*



*Fig. 3.*



*Fig. 4.*



INVENTORS

James E. Little,  
Frank O. Kichline  
and August Ehrgott.  
R. S. C. Dougherty  
ATTORNEY

May 31, 1932.

J. E. LITTLE ET AL

1,860,811

TREATMENT OF ORES

Filed May 26, 1926

2 Sheets-Sheet 2



Fig. 5.



Fig. 6.

INVENTORS  
James E. Little,  
Frank O. Kickline  
BY and August Ehrgott.  
R. S. C. Dougherty. ATTORNEY

## UNITED STATES PATENT OFFICE

JAMES E. LITTLE, OF BETHLEHEM, AND FRANK O. KICHLIN AND AUGUST EHRGOTT, OF LEBANON, PENNSYLVANIA, ASSIGNEES TO BETHLEHEM STEEL COMPANY

## TREATMENT OF ORES

Application filed May 26, 1928. Serial No. 111,879.

This invention relates to a method of dressing ores which exist in nature in a state of subdivision, as for example, earthy ferruginous ores, such as limonite and turgite and which have ores of other metals associated with them, as for example chromite. Hitherto it has not been found practicable to separate these ores by the normal methods well known to ore dressing practice.

Our invention has for an object a process for treating complex ores, in which the individual ore components and the gangue are intimately associated and are in a condition of natural subdivision, in order that said ores may be adapted to normal methods of separation.

As a specific example of this problem there may be mentioned certain chromiferous iron ores of Cuba, containing about 2% of metallic chromium in the form of chromite, which latter it is desirable to separate as a concentrate for the manufacture of ferro alloys.

In these ores the limonite, turgite and gangue constituents, such as alumina, for example, are in an earthy or clay-like condition. The chromite, on the other hand is in a relatively granular or "sandy" condition, and is also rather brittle.

These chromiferous iron ores have hitherto been submitted to a nodulizing process, wherein the finely divided material is dried and agglomerated to a condition suitable for the blast furnace; in this manner a chromiferous pig iron has been obtained suitable for special purposes. But no satisfactory process has yet been developed whereby the chromite could be separated from the limonite and the gangue of the ore, so as to result in any degree of concentration of the chromium bearing material.

After protracted experiments with all the methods of ore separation known in the art, none of which proved successful in the treatment of this particular chromiferous iron ore, we discovered that a washing process in which the ore could be subjected to a moderate degree of rubbing or of softened abrasion, but not of so violent a character as to break up particles of chromite, is very beneficial to the

ore and permits of a substantial separation of limonite and chromite by normal methods of ore separation.

The treatment towards which our invention is directed is that, which may be obtained by rubbing the particles of ore with the fingers under water in a miner's pan, and overflowing the particles of limonite which tend to disperse in the water, leaving the chromite in the residue of the pan. The effect sought is to rub and wash off the clayey limonite and similar clayey constituents from the "sandy" or granular constituents such as chromite, without substantially effecting the condition of this brittle constituent. Various means may be utilized for reproducing this effect on a practical scale, such as by passing a pulp of ore in water through a ball or rod mill, in which the balls or rods are formed of or encased in rubber. Alternatively any suitable means of agitation may be used which will not substantially disintegrate the chromite particles, as for example agitators having soft or flexible paddles or agitators containing rubber balls or materials of a similarly flexible character, the agitated pulp being then passed to a classifier or to a hydroseparator for separation of the limonite. The functions of agitation and classification may likewise be combined in a single apparatus where the nature of the ore permits, as for example in a classifier of the rake type, but equipped with soft or flexible raking edges.

In order to illustrate the nature of means suitable for carrying out our process, we show in Figure 1 a sectional elevation of a ball mill of conventional type having balls encased in rubber;

In Fig. 2 a part sectional elevation of a rod mill having rods encased in rubber;

In Fig. 3 a sectional elevation of an agitator having rubber balls mixed with the ore pulp;

In Fig. 4 a cross section of the scoop provided in a conventional ball mill;

In Fig. 5 a rake type classifier, having rubber or similarly flexible strips attached to the edges of the rakes; and

In Fig. 6 an enlarged section of a portion of the rake.

Referring to the drawings, we show in Fig. 1 a ball mill 11 of conventional type having driving gear 13, feed scoop 14, a feed launder 15 and balls encased in rubber 16. In Fig. 2, we show a portion of a rod mill 11, having a driving gear 18 and rods encased with rubber 17.

As previously set forth, the degree of attrition effected in these mills, whether they be loaded with balls or with rods is modified by the fact that they are encased in flexible material, as for example rubber. This probably results in deadening the effect normally produced by the cascading of the balls (or rods) in the mill and therefore limits their influence entirely to one of softened abrasion with a minimum of attrition.

In Fig. 3, we show an apparatus of somewhat different character to those above described, but susceptible of effecting a similar result. In this figure we show a tank 21 having rotatable agitating means 23, feed launder 24 an overflow launder 25, a discharge outlet 26 and flexible surfaced balls, as for example rubber balls 27. An apparatus such as that indicated in this figure is of the general character of a clay "blunger".

As our process contemplates the steps of gentle abrasion to be followed by normal methods of hydroseparation, it will be obvious that these steps may be combined in one apparatus. We therefore show in Fig. 5 a single-deck rake classifier 30 of well known type having a plurality of rakes 31, the edges 32 of which are provided with overhanging strips 33 of rubber, leather, or other material of a similarly flexible character. The working position of the rake mechanism in respect to the tank bottom is adjustable, by the means normally provided in this type of apparatus. A suitable method of fastening the strips to the edges of the rakes is shown in Fig. 6.

It will be apparent that in this process the aim is not to grind or crush any of the constituents but to rub and simultaneously wash the clayey constituents from the granular or sandy. This we secure by rubbing with cushioned elements in the presence of excess of water to remove the clayey from the sandy constituents.

By following the methods outlined above and using apparatus of the general types illustrated in the drawings, we have been able to separate 90% of the ore, as an overflow containing only a small proportion of chromite, from a residue or underflow containing a substantial proportion of chromium and which may be further concentrated.

For example, an ore of the following analysis:

|    |       |
|----|-------|
| Fe | 51.81 |
| Ni | 1.84  |
| Cr | 2.05  |
| Co | .18   |

treated in the manner described yields an overflow containing 90% of the ore, analyzing Fe 49.95 and Cr .77. The residue on drying and screening shows approximately 20% of plus 40 mesh and 12% of minus 300 mesh, said plus 40 mesh material being mainly limonite and the remainder containing chromite. The whole of this residue when recycled through the washing agitator and hydroseparated, to further eliminate the coarse limonite, analyzed 38% of chromium sesquioxide, equivalent to 26% of metallic chromium and 22% of Ferric oxide. The final yield of chromium bearing residue represents about 3 1/2% of the original ore. The overflow solids may be nodulized and used in the blast furnace in the usual manner. The dried residue is suitable for normal reduction in an electric furnace.

From the above it will be evident that we have devised a process, whereby earthy ferruginous ores and the like may now be separated in a substantial degree from other finely sub-divided ores intimately associated with them. The chromiferous iron ore, above referred to as an example of our process, is but one of many complex ores which are amenable to this treatment.

It will be obvious to those skilled in the art, that our invention is susceptible of various changes and modifications without departing from the spirit thereof and we desire therefore that only such limitations shall be placed thereupon as are imposed by the prior art or as are specifically set forth in the appended claim.

Having thus described our invention, what we claim as new and desire to secure by Letters Patent is:

In a process for treating ores comprising limonite and chromite, the steps of subjecting such ores to substantially freely resilient attritive impacts while in substantially free suspension in liquid, said impacts proportioned to disintegrate the limonite but not the chromite and separating the so differentially disintegrated ingredients.

In testimony whereof we hereunto affix our signatures.

JAMES E. LITTLE.  
FRANK O. KICHLINE.  
AUGUST EHRGOTT.

115

116

117

120

125

130